

Dec. 4, 1928.

1,694,265

**G. E. INMAN**

## METHOD AND APPARATUS FOR TREATING FILAMENTS

Filed May 10, 1926

Fig. 1



Fig. 2



Fig. 3



卷之三

INVENTOR:  
GEORGE E. INMAN,

Alexander S. Ladd.

His ATTORNEY.

Patented Dec. 4, 1928.

1,694,265

# UNITED STATES PATENT OFFICE.

GEORGE E. INMAN, OF EAST CLEVELAND, OHIO, ASSIGNOR TO GENERAL ELECTRIC COMPANY, A CORPORATION OF NEW YORK.

## METHOD AND APPARATUS FOR TREATING FILAMENTS.

Application filed May 10, 1926. Serial No 107,883.

My invention relates to methods and apparatus for applying coatings to very fine wires, and more specifically to methods and apparatus for applying so-called "getters" 5 to coiled filaments for incandescent lamps and similar devices. Getters are chemicals which are introduced into incandescent lamps or similar devices for the purpose of improving the performance of the lamp as 10 by improving the vacuum in the case of vacuum devices or by combining with metallic vapors and preventing injurious discoloration of the bulb. Heretofore it has been 15 the practice in the case of coiled filaments to apply the getter by dipping the filaments in a getter solution. The dipping method is slow and messy by comparison with my method, and has not produced as uniform results. Further features and advantages 20 of my invention will appear from a description of a species thereof.

In the drawing Fig. 1 is a perspective of an apparatus embodying my invention; Fig. 2 is an elevation partially in section of the 25 tube for the getter solution; Fig. 3 is an enlarged plan view of the filament container; and Fig. 4 is an enlarged view of a coiled filament.

As shown in the drawing, the filament 30 coil container 10 ordinarily of glass is in the form of a cylinder open at one end and adapted to contain a quantity of filament coils 11. The other end is closed except for the two tubulures 12 and 13. The container 35 10 is supported in an inclined position, preferably about 45°, and is held by a strap 14 on a slide 15 which engages the parallel guides 16 and 17 on a supporting block 18 carried by a base 19. There are two air jets 40 20 and 21 disposed opposite the open ends of the tubulures 12 and 13 respectively. The getter solution is carried in a tube 22 which may be graduated. The lower end of the tube carries a metal end piece 23 which has 45 an outlet nozzle 24. A needle valve 25 preferably of brass projects through said nozzle and at its upper end has a head 26 projecting above the metal upper end piece 26' of the tube. An adjustable cap 27 bears against 50 the said needle holder and the opening of the nozzle 24 may be regulated by means of this cap as the said needle head is provided with an extension 27' surrounded by the spring 27" which serves to keep the top of

the holder against the said cap 27. The getter solution may be supplied through funnel 28 preferably of brass communicated with the inlet pipe 29. The rate of flow of the getter solution may be regulated by adjusting needle 25 through the cap 27. The 55 getter tube is supported by the brackets 30 and 31 and carried by a standard 32. The air jets 20 and 21 and the air supply pipe connected thereto are supported by a bracket 33 adjustably mounted on a block 34 which 60 is adjustably supported on an extension from the bracket 31.

The jet 21 and the corresponding tubulure 13 are disposed tangentially of the cylinder 10. The air issuing from the jet 21 65 serves therefore to whirl the coils rapidly around the bottom of the container. At the same time the air issuing from the jet 20 encounters the getter solution issuing from the nozzle 24 and directs it into the tubulure 70 75 12 to be sprayed upon the whirling coils. A receptacle 35 is provided to receive any excess of the getter solution which may flow from tubulure 13. The mounting of container 10 is preferably such that tubulure 80 85 13 is substantially horizontal and this prevents accumulation of liquid in the container. A ventilator 36 is provided with a suitable exhaust connection to take off the dust and vapors while the apparatus is in 90 operation. The air pressure for the jets 20 and 21 is preferably high. About thirty-five pounds has been found to be suitable. In adjusting the needle 25, the point should be opposite the center of the tubulure 12. 95 The coils are weighed before and after gettering so as to make sure that the proper amount of getter has been applied. The character of the getter solution and the amount of air pressure are such that the 100 coils do not become wet but are merely moist. If allowed to become wet, the coils would stick together and fail to rotate and hence would be improperly coated. The getter material, for instance powdered cryolite, is 105 in suspension in a volatile carrier. One solution which has been used was made by adding 200 grams of the powdered getter material to 150 grams of lacquer containing amyl acetate and then diluting by adding four parts of a mixture of 80% methyl alcohol and 20% ether. The presence of the combination of a quick drying carrier such

as the alcohol and ether mixture with a relatively slow drier such as the amyl acetate is desirable.

- It will be apparent that after a trial the proper adjustments can be made. As a rule the getter flows at the rate of two or three cubic centimeters per minute while .4 of a cubic centimeter of mixture is usually required for a gram of twenty-five watt coils, and about .7 of a cubic centimeter for a gram of fifty watt coils to give the correct percentage. As the head of getter decreases in the tube, the adjusting cap can be slightly turned to keep the flow constant.
- When the predetermined quantity of getter has been applied, the getter needle is shut down. Then the air is closed off and the coils are removed and weighed. If the weight is too high, the coils are returned to the gettering vessel and the air is turned on to rotate the coils for a few seconds. This rubs off some of the getter. If the percentage is too low, more getter may be sprayed on without removing the previous coating.

What I claim as new and desire to secure

by Letters Patent of the United States, is:—

1. The method of applying getter to filaments for electric incandescent lamps and similar articles which consists in placing a number of said filaments in a receptacle so that they are supported on the bottom thereof, and then spraying the getter material upon said filaments and at the same time directing gas pressure tangentially so as to cause a swirling of said filaments in front of the spray.

2. In an apparatus for applying material to filaments, the combination of a receptacle for holding a number of filaments and having a plurality of openings in its wall near the bottom thereof, a gas pressure jet disposed at each of said openings at least one of which is directed tangentially of the receptacle, and means for feeding a liquid containing said material so as to be encountered by the gas issuing from at least one of said jets and sprayed into the corresponding opening.

In witness whereof, I have hereunto set my hand this 7th day of May, 1926.

GEORGE E. INMAN.